

(Specimens.)

J. A. PEASE & G. J. BABSON.

PAPER PULP FABRIC FOR BOXES, &c.

No. 314,054.

Patented Mar. 17, 1885.



Fig. 1.



Fig. 2.

Witnesses:

Louis C. Halls,  
Wm. Duray

Inventors:

Julius A. Pease <sup>and</sup>  
George J. Babson  
By E. B. Stetson  
Attorney.

# UNITED STATES PATENT OFFICE.

JULIUS A. PEASE, OF WEST MEDFORD, AND GEORGE J. BABSON, OF BOSTON, MASSACHUSETTS.

## PAPER-PULP FABRIC FOR BOXES, &c.

SPECIFICATION forming part of Letters Patent No. 314,054, dated March 17, 1885.

Application filed January 13, 1885. (Specimens.)

*To all whom it may concern:*

Be it known that we, JULIUS A. PEASE and GEORGE J. BABSON, citizens of the United States, residing, respectively, at West Medford and Boston, in the counties of Middlesex and Suffolk and State of Massachusetts, have invented certain new and useful Improvements in Fabrics, of which the following is a specification, reference being had to the accompanying drawings.

The object of this invention is to provide a fabric or material for various purposes, especially for the purpose of making articles which require in their use or which can advantageously possess the characteristics of paper, and at the same time possess the quality of strength in a degree far in excess of that of paper.

It is well known that paper has been applied to many uses in the mechanic arts by reason of its peculiar texture, pliability, submission to manipulation, and cheapness, and that by the application thereto of waterproofing and fireproofing compounds it is rendered capable of use in exposed positions, and that by excessive pressure it is rendered capable of resisting great wear; but with all these advantages in use it lacks strength to such a degree as will permit of its use under certain conditions requiring a capability of resisting strain in various directions.

Heretofore finished paper in sheets has been applied and secured to sheet metal upon one or both sides thereof in order to secure the advantages which constitute a part of the object of our invention; but in such cases the material resulting from such a combination of the substances mentioned has usually been limited in area and outline to that of the article made from such compound material, and in a degree necessarily so by reason of the limited area of the sheet metal to be obtained for association with the paper. Furthermore, in such cases finished paper alone has been combined with strengthening materials, and always with an intervening cement or adhesive agent.

By our invention we are enabled to produce a fabric or material, either in continuous webs or lengths of desired widths, which possesses all the characteristics of paper, and at the same

time the strength of metallic materials. We accomplish this result—the production of such a material—by using as the base or foundation thereof wire-cloth of a desired mesh, fineness, or coarseness in the strands thereof, and as the outer portions of said material we employ paper-pulp. We combine with a continuous web of wire-cloth continuous webs of pulp in such manner that the pulp is forced through the meshes of the wire-cloth, and completely envelops and covers the same, so that in outward appearance the material is exactly like that of paper of the same texture and quality, while it is at the same time capable of being rolled into rolls for shipment and transportation, to be unrolled for use in continuous sheets or in parts thereof, which may be cut in any desired shape for the manufacture of desired articles, especially those which can be struck up or formed without seam, while those requiring seams may be provided with the same at desired points, and the parts secured together by paste or cement, as in ordinary paper articles. The cementation of joints in our material is assured by reason of the fact that all points on its outer surfaces are of pulp. Again, such material is capable of being ornamented by the application thereto of finished paper or other material, or by the finishing the surface of the pulp itself, varnishing, painting, or treating with any suitable finishing, waterproofing, or fireproofing compound, or in the latter case of combining with the pulp itself of asbestos in the usual well-known proportions.

Our invention therefore consists in a fabric or material, in a continuous sheet or in roll form, which consists of wire-cloth embedded or completely covered with paper-pulp.

Referring to the drawings, Figure 1 represents a roll of fabric or material or compound paper made in accordance with our invention, and Fig. 2 is a transverse vertical section of the same.

Like letters refer to like parts in both figures.

A represents any suitable pulp, and B represents the wire-cloth embedded therein.

For the purpose of disclosing one method or manner of making our material, which method and manner is not claimed herein, as it will

constitute the subject-matter of a separate application, we deem it proper to state that we employ a paper-making machine which is constructed and adapted to deliver to any desired point two independent webs or continuous sheets of pulp, at which point these sheets pass through any suitable pressure-rollers, so as to be formed into a single sheet or web. At a point in the machine which is to the rear or back of (in the line of feed) said pressure-rollers we provide means for supporting the continuous sheet or web or wire-cloth in roll form, and conduct by hand or suitable devices the leading end of said cloth into, between, and through the said pressure-rollers, and between the two continuous sheets or webs of pulp passing thereinbetween, so that by the pressure-rollers we compress continuous sheets of pulp against the opposite surfaces and into and through the meshes of the wire-cloth, which may or may not, as desired, be first waterproofed to prevent rusting. After passing through said rolls, the fabric is delivered to any suitable drying mechanism, and subsequently from the machine as wire-cloth completely covered and embedded with pulp.

We find this fabric or material sufficiently flexible for all purposes to which any other material of this nature is adapted, and we also find it susceptible of division into sections of desired area and contour for special purposes.

We deem it proper to state that our invention consists in the fabric or material herein described irrespective of any method of manufacturing the same, because still other methods may be devised than that specified, such as interposing independent squares or pieces

other than continuous sheets of wire-cloth between the sheets of pulp.

We are aware that heretofore a wire form of an article has been made and the same completely covered with pulp, to produce the article in accordance with the shape or form made of wire, and we do not therefore broadly claim covering wire with pulp; but

What we claim, and desire to secure by Letters Patent, is—

1. As an article of manufacture, a compound material consisting of wire-cloth completely embedded and covered with pulp, substantially as specified.

2. A continuous sheet, roll, or web of material consisting of wire-cloth embedded and completely covered with paper-pulp, substantially as specified.

3. The method of making the compound fabric or material herein specified, which consists in uniting by compression continuous sheets or webs of pulp and of wire-cloth in such manner as to completely cover and embed the latter in and by the former, substantially as specified.

4. As an article of manufacture, the fabric or material herein described, consisting of wire-cloth rendered water-repellent and covered and having its meshes filled with pulp, substantially as specified.

In testimony whereof we have affixed our signatures in presence of two witnesses.

JULIUS A. PEASE.  
GEO. J. BABSON.

Witnesses:

CHARLES B. HUGHES,  
GILBERT COLLINS.